# EUROPEAN PATENT SPECIFICATION

(11) **EP 2 432 919 B1**
(45) Date of publication and mention of the grant of the patent: **24.07.2013**
(21) Application number: 10720911.6
(22) Date of filing: 18.05.2010
(51) Int. Cl.: C25B 11/06, C25B 11/04

(54) **CATHODE FOR ELECTROLYTIC PROCESSES**
KATHODE FÜR ELEKTROLYTISCHE VERFAHREN
CATHODE DESTINÉE À DES PROCESSUS ÉLECTROLYTIQUES

(30) Priority: 19.05.2009 IT MI20090880
(43) Date of publication of application: 28.03.2012
(73) Proprietor: Industrie De Nora S.P.A., 20134 Milano (IT)
(72) Inventor: BRICHESE, Marianna, I-30021 Caorle (IT); ANTOZZI, Antonio, Lorenzo, I-23807 Merate (IT); CALDERARA, Alice, I-26020 Agnadello (IT)
(74) Representative: Reitstötter - Kinzebach
(86) International application number: PCT/EP2010/056797
(87) International publication number: WO 2010/133583

(56) References cited:
- US-A- 4 377 454
- US-A- 4 798 662
- DATABASE CA [Online] CHEMICAL ABSTRACTS SERVICE, COLUMBUS, OHIO, US; 2000, NAWRAT, GINTER ET AL: "Cathodes with active coatings with a reduced hydrogen discharge overvoltage" XP002555823 retrieved from STN Database accession no. 134:302107 & TECHNOLOGIA CHEMICZNA NA PRZELOMIE WIEKOW , 335-338 PUBLISHER: WYDAWNICTWO STALEGO KOMITETU KONGRESOW TECHNOLOGII CHEMICZNEJ, GLIWICE, POL. CODEN: 69AXVP, 2000,
- DATABASE WPI Week 1977 Thomson Scientific, London, GB; AN 55426y XP002555824 & SU 527 488 A1 (KUKOZ F I) 5 September 1976 (1976-09-05)

## Description

### FIELD OF THE INVENTION

The present invention relates to an electrode suitable for acting as cathode in electrolytic cells, for instance as hydrogen-evolving cathode in chlor-alkali cells.

### BACKGROUND OF THE INVENTION

The invention relates to an electrode for electrolytic processes, in particular to a cathode suitable for hydrogen evolution in an industrial electrolysis process. Reference will be made hereafter to chlor-alkali electrolysis as a typical industrial electrolytic process with cathodic evolution of hydrogen, but the invention is not limited to a particular application. In the electrolytic process industry, competitiveness is associated with several factors, the main one being the reduction of energy consumption, directly linked to the electrical operating voltage. Among the various components which contribute to determining the operating voltage, besides factors associated with ohmic drop and mass transport, the overvoltages of the evolution reactions of the two products, anodic and cathodic (in the case of chlor-alkali electrolysis, anodic chlorine evolution overvoltage and cathodic hydrogen evolution overvoltage) are of high relevance. In the industrial practice, such overvoltages are minimised through the use of suitable catalysts. The use of cathodes consisting of metal substrates, for instance of nickel, copper or steel, provided with catalytic coatings based on oxides of ruthenium, platinum or other noble metals is known in the art. US 4,465,580 and US 4,238,311 for instance disclose nickel cathodes provided with a coating based on ruthenium oxide mixed with nickel oxide, capable of lowering the cathodic hydrogen evolution overvoltage. Also other types of catalytic coating for metal substrates suitable for catalysing hydrogen evolution are known, for instance based on platinum, on rhenium or molybdenum optionally alloyed with nickel, on molybdenum oxide. The majority of these formulations nevertheless show a rather limited operative lifetime in common industrial applications, probably due to the poor adhesion of the coating to the substrate.

A certain increase in the useful lifetime of cathodes activated with noble metal at the usual process conditions is obtainable by depositing an external layer on top of the catalytic layer, consisting of an alloy of nickel, cobalt or iron with phosphorus, boron or sulphur, for example by means of an electroless procedure, as disclosed in US 4,798,662. Further, US 4,377, 454 describes a cathode having an intermediate coating for corrosion protection.

Such kind of finding however leaves totally unsolved the problem of tolerance to current reversals which sometimes may take place in the electrolysers, almost always due to unexpected malfunctioning, for instance during maintenance operations. In such a situation, the anchoring of the catalytic coating to the substrate is more or less seriously compromised, part of the active component being liable to detachments from the cathode substrate with consequent decrease of the catalytic efficiency and increase of the operating voltage. This phenomenon is particularly relevant in the case of cathodes containing ruthenium dioxide, which are vastly applied in industrial processes due to their excellent catalytic activity. A measure of such quick loss of activity can be detected, as it will be clear to a person of skill in the art, by subjecting electrode samples to cyclic voltammetry within a range of potential between hydrogen cathodic discharge and oxygen anodic one: an electrode potential decay in the range of tens of millivolts is almost always detectable since the very first cycles. This poor resistance to inversions constitutes an unsolved problem for the main types of activated cathode for electrolytic applications and especially for cathodes based on ruthenium oxide optionally in admixture with nickel oxide commonly employed in chlor-alkali electrolysis processes.

### SUMMARY OF THE INVENTION

Various aspects of the invention are set out in the accompanying claims.

In one embodiment, the present invention relates to an electrode suitable for functioning as cathode in electrolytic processes comprising a conductive substrate sequentially coated with a first protective intermediate layer, a catalytic layer and a second external protective layer, the first and the second protective layers comprising an alloy consisting of one or more metals selected between nickel, cobalt and chromium and one or more non-metals selected between phosphorus and boron; the alloy of the protective layers may additionally contain a transition element, for instance selected between tungsten and rhenium. In one embodiment, the catalytic layer contains oxides of non-noble transition metals, for instance rhenium or molybdenum. In one embodiment, the catalytic layer contains platinum group metals and oxides or compounds thereof, for instance ruthenium dioxide. The experimental tests showed that the deposition of compact and coherent layers of the above defined alloys externally to the catalytic layer and at the same time between catalytic layer and substrate favours the catalyst anchoring to a surprising extent, without the additional ohmic drop significantly affecting the electrode potential.

In one embodiment, at least one of the two protective layers consists of an alloy which can be deposited by autocatalytic chemical reduction according to the process known to those skilled in the art as "electroless". This type of manufacturing procedure can have the advantage of being easily applicable to substrates of various geometries such as solid, perforated or expanded sheets as well as meshes, optionally of very reduced thickness, without having to introduce substantial changes to the manufacturing process as a function of the various geometries and sizes, as would happen in the case of a galvanic deposition. The electroless deposition is suited to substrates of several kinds of metals used in the production of cathodes, for instance nickel, copper, zirconium and various types of steels such as stainless steels.

In one embodiment, the alloy which can be deposited via electroless is an alloy of nickel and phosphorous in a variable ratio, generally indicated as Ni-P.

In one embodiment, the specific loading of the first protective layer, that is the interlayer directly contacting the metal substrate, is lower, for instance being about one half, than the specific loading of the second outermost protective layer. In one embodiment, the specific loading of the interlayer is 5-15 g/m² and than the specific loading of the external protective layer is 10-30 g/m². The above specified loadings are sufficient to obtain macroscopically compact and coherent layers conferring a proper anchoring of the catalytic layer to the base and a protection from the aggressive action of the electrolyte, without hampering the mass transport of the same electrolyte to the catalytic sites and the release of hydrogen evolved by the cathodic reaction.

In one embodiment, a method for the preparation of a cathode as described comprises a step of deposition of the protective interlayer via electroless putting the substrate in contact for a sufficient time with a solution, gel or ionic liquid or sequentially with more solutions, gels or ionic liquids containing the precursors of the selected alloy; a subsequent step of deposition of the catalytic layer by application of a precursor solution of the catalytic components in one or more cycles with thermal decomposition after each cycle; a subsequent step of deposition of the external protective layer via electroless, analogous to the interlayer deposition step.

In one embodiment, a layer of nickel-phosphorous alloy can be deposited as the protective interlayer or external layer by sequential dipping in a first solution containing 0.1-5 g of PdCl₂ in acidic environment for 10-300 s; a second solution containing 10-100 g/l of NaH₂PO₂ for 10-300 s; a third solution containing 5-50 g/l of NaH₂PO₂ and optionally NiSO₄, (NH₄)₂SO₄ and Na₃C₃H₅O(CO₂)₃ in a basic environment of ammonia for 30 minutes - 4 hours.

In one embodiment, the catalyst precursor solution contains Ru(NO)ₓ(NO₃)₂ or RuCl₃.

Some of the most significant results obtained by the inventors are presented in the following examples, which are not intended as a limitation of the extent of the invention.

### EXAMPLE 1

A nickel mesh of 100 mm X 100 mm X 1 mm size was sandblasted, etched in HCl and degreased with acetone according to a standard procedure, then subjected to an electroless deposition treatment by sequential dipping in three aqueous solutions having the following composition:
- Solution A: 1 g/l PdCl₂ + 4 ml/l HCl
- Solution B: 50 g/l NaH₂PO₂
- Solution C: 20 g/l NiSO₄ + 30 g/l (NH₄)₂SO₄ + 30 g/l NaH₂PO₂ + 10 g/l Na₃C₃H₅O(CO₂)₃ (trisodium citrate) + 10 ml/l ammonia.

The mesh was sequentially dipped for 60 seconds in solution A, seconds in solution B and 2 hours in solution C.

At the end of the treatment, a superficial deposition of about 10 g/m² of Ni-P alloy was observed.

The same mesh was subsequently activated with a RuO₂ coating consisting of two layers, the former deposited in a single coat by application of RuCl₃ dissolved in a mixture of aqueous HCl and 2-propanol, followed by thermal decomposition, the latter deposited in two coats by application of RuCl₃ dissolved in 2-propanol, with subsequent thermal decomposition after each coat. The thermal decomposition steps were carried out in a forced ventilation oven with a thermal cycle of 10 minutes at 70-80°C and 10 minutes at 500°C. In this way, 9 g/m² of Ru expressed as metal were deposited.

The thus activated mesh was again subjected to an electroless deposition treatment by dipping in the three above indicated solutions, until obtaining the deposition of an external protective layer consisting of about 20 g/m² of Ni-P alloy.

Three samples of 1 cm² cut out from the activated mesh showed a starting IR-corrected average cathodic potential of -930 mV/NHE at 3 kA/m² under hydrogen evolution in 33% NaOH, at a temperature of 90°C, which indicates an excellent catalytic activity. The same samples were subsequently subjected to cyclic voltammetry in the range of -1 to + 0.5 V/NHE with a 10 mV/s scan rate; the average cathodic potential shift after 25 cycles was 35 mV, indicating an excellent current reversal tolerance.

From the same activated mesh, 3 samples of 2 cm² surface were also cut out to be subjected to an accelerated life-test under cathodic hydrogen evolution at exasperated process conditions, utilising 33% NaOH at 90°C as the electrolyte and setting a current density of 10 kA/m². The test consists of periodically detecting the cathodic potential, following its evolution over time and recording the deactivation time. The latter is defined as time required to reach a potential increase of 100 mV with respect to the starting value. The average deactivation time of the three samples was 3670 hours.

### EXAMPLE 2

A nickel mesh of 100 mm X 100 mm X 1 mm size was sandblasted, etched in HCl and degreased with acetone according to a standard procedure, then subjected to an electroless deposition treatment by dipping for 1 hour in an aqueous solution having the following composition: 35 g/l NiSO₄ + 20 g/l MgSO₄ + 10 g/l NaH₂PO₂ + 10 g/l Na₃C₃H₅O(CO₂)₃ + 10 g/l CH₃COONa.

At the end of the treatment, a superficial deposition of about 8 g/m² of Ni-P alloy was observed.

The same mesh was subsequently activated with a RuO₂ coating consisting of two layers, the former deposited in a single coat by application of RuCl₃ dissolved in a mixture of aqueous HCl and 2-propanol, followed by thermal decomposition, the latter deposited in two coats by application of RuCl₃ dissolved in 2-propanol, with subsequent thermal decomposition after each coat. The thermal decomposition steps were carried out in a forced ventilation oven with a thermal cycle of 10 minutes at 70-80°C and 10 minutes at 500°C. In this way, 9 g/m² of Ru expressed as metal were deposited.

The thus activated mesh was again subjected to an electroless deposition treatment by dipping in the above indicated solution, until obtaining the deposition of an external protective layer consisting of about 25 g/m² of Ni-P alloy.

Three samples of 1 cm² cut out from the activated mesh showed a starting IR-corrected average cathodic potential of -935 mV/NHE at 3 kA/m² under hydrogen evolution in 33% NaOH, at a temperature of 90°C. The same samples were subsequently subjected to cyclic voltammetry in the range of -1 to + 0.5 V/NHE with a 10 mV/s scan rate; the average cathodic potential shift after 25 cycles was 35 mV, indicating an excellent current reversal tolerance.

From the same activated mesh, 3 samples of 2 cm² surface were also cut out to be subjected to the same accelerated life-test described in example 1. The average deactivation time of the three samples was 3325 hours.

### EXAMPLE 3

Example 1 was repeated on a nickel mesh of 100 mm X 100 mm X 0.16 mm size after adding a small amount of a thickener (xanthan gum) to solutions A and B, and of the same component to a solution equivalent to C but with all solutes in a threefold concentration. Brush-applicable homogeneous gels were obtained in the three cases.

The three gels were sequentially applied to the nickel mesh, until obtaining a superficial deposition of about 5 g/m² of Ni-P alloy.

The same mesh was subsequently activated with a RuO₂ coating consisting of two layers, the former deposited in a single coat by application of RuCl₃ dissolved in a mixture of aqueous HCl and 2-propanol, followed by thermal decomposition, the latter deposited in two coats by application of RuCl₃ dissolved in 2-propanol, with subsequent thermal decomposition after each coat. The thermal decomposition steps were carried out in a forced ventilation oven with a thermal cycle of 10 minutes at 70-80°C and 10 minutes at 500°C. In this way, 9 g/m² of Ru expressed as metal were deposited.

The three above gels were again sequentially applied to the thus activated mesh, until obtaining the superficial deposition of about 10 g/m² of Ni-P alloy.

Three samples of 1 cm² cut out from the activated mesh showed a starting IR-corrected average cathodic potential of -936 mV/NHE at 3 kA/m² under hydrogen evolution in 33% NaOH, at a temperature of 90°C. The same samples were subsequently subjected to cyclic voltammetry in the range of -1 to + 0.5 V/NHE with a 10 mV/s scan rate; the average cathodic potential shift after 25 cycles was 38 mV, indicating an excellent current reversal tolerance.

From the same activated mesh, 3 samples of 2 cm² surface were also cut out to be subjected to the same accelerated life-test described in example 1. The average deactivation time of the samples was 3140 hours.

### COMPARATIVE EXAMPLE 1

A nickel mesh of 100 mm X 100 mm X 1 mm size was sandblasted, etched in HCl and degreased with acetone according to a standard procedure, then directly activated without applying any protective interlayer with a RuO₂ coating consisting of two layers with a total loading of 9 g/m² of Ru expressed as metal, according to the previous examples.

Three samples of 1 cm² cut out from the activated mesh showed a starting I R-corrected average cathodic potential of -928 mV/NHE at 3 kA/m² under hydrogen evolution in 33% NaOH, at a temperature of 90°C. The same samples were subsequently subjected to cyclic voltammetry in the range of -1 to + 0.5 V/NHE with a 10 mV/s scan rate; the average cathodic potential shift after 25 cycles was 160 mV, indicating a non-optimum current reversal tolerance.

From the same activated mesh, 3 samples of 2 cm² surface were also cut out to be subjected to the same accelerated life-test described in example 1. The average deactivation time of the samples was 2092 hours.

### COMPARATIVE EXAMPLE 2

A nickel mesh of 100 mm X 100 mm X 1 mm size was sandblasted, etched in HCl and degreased with acetone according to a standard procedure, then directly activated without applying any protective interlayer with a RuO₂ coating consisting of two layers with a total loading of 9 g/m² of Ru expressed as metal, according to the previous examples.

The thus activated mesh was subjected to an electroless deposition treatment by dipping in the three solutions of Example 1, until obtaining the superficial deposition of an outer protective layer consisting of about 30 g/m² of Ni-P alloy.

Three samples of 1 cm² cut out from the activated mesh showed a starting IR-corrected average cathodic potential of -927 mV/NHE at 3 kA/m² under hydrogen evolution in 33% NaOH, at a temperature of 90°C. The same samples were subsequently subjected to cyclic voltammetry in the range of -1 to + 0.5 V/NHE with a 10 mV/s scan rate; the average cathodic potential shift after 25 cycles was 60 mV, indicating a non-optimum current reversal tolerance.

From the same activated mesh, 3 samples of 2 cm² surface were also cut out to be subjected to the same accelerated life-test described in example 1. The average deactivation time of the samples was 2760 hours.

The previous description is not intended to limit the invention, which may be used according to different embodiments without departing from the scopes thereof, and whose extent is univocally defined by the appended claims.

Throughout the description and claims of the present application, the term "comprise" and variations thereof such as "comprising" and "comprises" are not intended to exclude the presence of other elements or additives.

The discussion of documents, acts, materials, devices, articles and the like is included in this specification solely for the purpose of providing a context for the present invention.

## Claims

1. Cathode suitable for hydrogen evolution in electrolytic processes comprising a conductive substrate coated with a first intermediate protective layer, a catalytic layer and a second external protective layer, said first and second protective layer comprising an alloy consisting of at least one metal selected between nickel, cobalt and chromium, at least one non-metal selected between phosphorus and boron and optionally a transition element selected between tungsten and rhenium.

2. The cathode according to claim 1 wherein said catalytic layer comprises at least one element selected from the group consisting of molybdenum, rhenium and platinum group metals.

3. The cathode according to claim 2 wherein said catalytic layer contains RuO₂.

4. The cathode according to any one of the previous claims wherein at least one of said first and said second protective layer comprises an alloy of nickel and phosphorus.

5. The cathode according to any one of the previous claims wherein said conductive substrate is a solid, punched on expanded sheet or a mesh made of nickel, copper, zirconium or stainless steel.

6. The cathode according to any one of the previous claims wherein said first protective layer has a specific loading of 5-15 g/m² and said second protective layer has a specific loading of 10-30 g/m².

7. Method for manufacturing a cathode according to any one of claims 1 to 6 comprising the steps of:
a) electroless deposition of said first protective layer by contacting said conductive substrate with at least one first solution, gel or ionic liquid containing the precursors of said alloy
b) application of said catalytic layer by thermal decomposition of at least one catalyst precursor solution in one or more cycles
c) electroless deposition of said second protective layer by contacting said conductive substrate provided with a catalytic layer with at least one second solution, gel or ionic liquid containing the precursors of said alloy.

8. The method according to claim 7 wherein at least one of said at least one first and said at least one second solution containing the precursors of said alloy contains NaH₂PO₂.

9. The method according to claim 7 wherein said deposition of said first and/or of said second protective layer is carried out by sequential dipping in:
a) a first solution containing 0.1-5 g of PdCl₂ in acidic environment for 10-300 s;
b) a second solution containing 10-100 g/l of NaH₂PO₂ for 10-300 s;
c) a third solution containing 5-50 g/l of NaH₂PO₂ and optionally NiSO₄, (NH₄)₂SO₄ and Na₃C₃H₅O(CO₂)₃ made alkaline by ammonia for 0.5-4 hours.

10. The method according to any one of claims 7 to 9 wherein said at least one catalyst precursor solution contains Ru(NO)ₓ(NO₃)₂ or RuCl₃.

## Patentansprüche

1. Kathode geeignet für Wasserstoffentwicklung in elektrolytischen Prozessen, welche ein leitendes Substrat, welches mit einer ersten schützenden Zwischenschicht beschichtet ist, eine katalytische Schicht und eine zweite schützende Außenschicht umfasst, wobei die erste und die zweite schützende Schicht eine Legierung, welche aus zumindest einem Metall ausgewählt zwischen Nickel, Kobalt und Chrom, zumindest einem NichtMetall ausgewählt zwischen Phosphor und Bor und optional einem Übergangselement ausgewählt zwischen Wolfram und Rhenium besteht.

2. Kathode nach Anspruch 1, wobei die katalytische Schicht zumindest ein Element ausgewählt aus der Gruppe bestehend aus Molybdän-, Rhenium- und Platingruppenmetallen umfasst.

3. Kathode nach Anspruch 2, wobei die Zwischenschicht RuO₂ enthält.

4. Kathode nach einem der vorhergehenden Ansprüche, wobei zumindest eine der ersten und der zweiten schützenden Schicht eine Legierung aus Nickel und Phosphor umfasst.

5. Kathode nach einem der vorhergehenden Ansprüche, wobei das leitende Substrat ein fester Stoff ist, welcher auf ein ausgedehntes Blech gestanzt ist oder welcher ein Netz aus Nickel, Kupfer, Zirkonium oder Edelstahl ist.

6. Kathode nach einem der vorhergehenden Ansprüche, wobei die erste schützende Schicht eine spezifische Beladung von 5-15 g/m² und die zweite schützende Schicht eine spezifische Beladung von 10-30 g/m² aufweist.

7. Verfahren zum Herstellen einer Kathode nach einem der Ansprüche 1 bis 6 umfassend die Schritte:
a) stromloses Abscheiden der ersten schützenden Schicht durch das Kontaktieren des leitenden Substrats mit zumindest einer ersten Lösung, Gel oder ionischen Flüssigkeit, welche die Ausgangsstoffe der Legierung enthalten
b) Auftragen der katalytischen Schicht zumindest einer katalytischen Ausgangsstofflösung in einem oder mehreren Zyklen durch Thermolyse
c) stromloses Abscheiden der zweiten schützenden Schicht durch Kontaktieren des leitenden Substrats ausgestattet mit einer katalytischen Schicht mit zumindest einer zweiten Lösung, Gel oder ionischen Flüssigkeit, welche die Ausgangsstoffe der Legierung enthalten.

8. Verfahren nach Anspruch 7, wobei zumindest eine der zumindest einen ersten und zumindest einen zweiten Lösung, welche die Ausgangsstoffe der Legierung enthält, NaH₂PO₂ enthält.

9. Verfahren nach Anspruch 7, wobei das Abscheiden der ersten und/oder zweiten schützenden Schicht ausgeführt wird durch sequentielles Eintauchen in:
a) eine erste Lösung, welche 0,1-5 g PdCl₂ in säurehaltiger Umgebung enthält, für 10-300 s;
b) eine zweite Lösung, welche 10-100 g/l NaH₂PO₂ enthält, für 10-300 s;
c) eine dritte Lösung, welche 5-50 g/l NaH₂PO₂ und optional NiSO₄, (NH₄)₂SO₄ und Na₃C₃H₅O(CO₂)₃ durch Ammoniak alkalisch gemacht enthält, für 0,5-4 Stunden.

10. Verfahren nach einem der Ansprüche 7 bis 9, wobei zumindest eine katalytische Ausgangsstofflösung Ru(NO)ₓ(NO₃)₂ oder RuCl₃ enthält.

## Revendications

1. Cathode appropriée pour un dégagement d'hydrogène dans des processus électrolytiques, comprenant un substrat conducteur revêtu d'une première couche protectrice intermédiaire, d'une couche catalytique et d'une seconde couche protectrice externe, lesdites première et seconde couches protectrices comprenant un alliage composé d'au moins un métal sélectionné parmi le nickel, le cobalt et le chrome, au moins un composé non métallique sélectionné parmi le phosphore et le bore et en option un élément de transition sélectionné parmi le tungstène et le rhénium.

2. Cathode selon la revendication 1, dans laquelle ladite couche catalytique comprend au moins un élément sélectionné dans le groupe composé de métaux du groupe du molybdène, du rhénium et du platine.

3. Cathode selon la revendication 2, dans laquelle ladite couche catalytique contient RuO₂.

4. Cathode selon l'une quelconque des revendications précédentes, dans laquelle au moins une desdites première et seconde couches protectrices comprend un alliage de nickel et de phosphore.

5. Cathode selon l'une quelconque des revendications précédentes, dans laquelle ledit substrat conducteur est un solide, une feuille perforée ou expansée ou un treillis fait de nickel, de cuivre, de zirconium ou d'acier inoxydable.

6. Cathode selon l'une quelconque des revendications précédentes, dans laquelle ladite première couche protectrice a une charge spécifique de 5 à 15 g/m² et ladite seconde couche protectrice a une charge spécifique de 10 à 30 g/m².

7. Procédé de fabrication d'une cathode selon l'une quelconque des revendications 1 à 6, comprenant les étapes de :
a) dépôt autocatalytique de ladite première couche protectrice par mise en contact dudit substrat conducteur avec au moins une première solution, ou un premier gel ou liquide ionique contenant les précurseurs dudit alliage,
b) application de ladite couche catalytique par décomposition thermique d'au moins une solution de précurseur de catalyseur en un ou plusieurs cycles,
c) dépôt autocatalytique de ladite seconde couche protectrice par mise en contact dudit substrat conducteur muni d'une couche catalytique avec au moins une seconde solution, ou un second gel ou liquide ionique contenant les précurseurs dudit alliage.

8. Procédé selon la revendication 7, dans lequel au moins une parmi ladite première, au moins au nombre de une, et ladite seconde, au moins au nombre de une, solutions contenant les précurseurs dudit alliage contient NaH₂PO₂.

9. Procédé selon la revendication 7, dans lequel ledit dépôt de ladite première et/ou ladite seconde couches protectrices est réalisé par trempage séquentiel dans :
a) une première solution contenant 0,1 à 5 g de PdCl₂ dans un environnement acide, pendant 10 à 300 s ;
b) une seconde solution contenant 10 à 100 g/l de NaH₂PO₂, pendant 10 à 300 s ;
c) une troisième solution contenant 5 à 50 g/l de NaH₂PO₂ et en option NiSO₄, (NH₄)₂SO₄ et Na₃C₃H₅O(CO₂)₃ rendue alcaline par de l'ammoniac, pendant 0,5 à 4 heures.

10. Procédé selon l'une quelconque des revendications 7 à 9, dans lequel ladite solution de précurseur de catalyseur, au moins au nombre de une, contient Ru(NO)ₓ(NO₃)₂ ou RuCl₃.
